

## UNITED STATES PATENT OFFICE

2,411,145

## INGREDIENTS FOR PRODUCING HIGH EXPLOSIVES

Michele Bonotto, Princeton, N. J., assignor to  
Dorothy Di Frasso, Beverly Hills, Calif.

No Drawing. Application December 15, 1941,  
Serial No. 423,038

5 Claims. (Cl. 260—112)

1

This invention relates to improvements in ingredients for producing high explosives and high explosives made therewith.

One of the objects of this invention is to utilize as an ingredient of an explosive a nitro-protein complex derived, provided by or obtained in either separated or combined form, from a nitrated vegetable material from which oil has been extracted and which is capable of being mixed with explosives having inherent explosive characteristics or with an oxygen-carrying substance for the purpose of producing a high explosive.

Still another objective of my invention is to utilize as an ingredient of an explosive a nitro-protein complex obtained or derived from a nitrated oil-bearing vegetable material from which oil has been extracted and which has a high protein content.

Still another object of my invention is to utilize as an ingredient of an explosive a nitro-protein complex derived from a nitrated oil-bearing vegetable material from which oil has been extracted and which has, in the wet basis, a protein content of the order of thirty percent (30%) to sixty-five percent (65%).

Still another object of my invention is to utilize as an ingredient of an explosive a nitro-protein complex procured from a nitrated vegetable material obtained from any one of an edible oil group of oil-bearing materials hereinafter more particularly defined and from which oil has been extracted.

Still another object of my invention is to utilize as an ingredient of an explosive a nitro-protein complex embodied in nitrated oil-bearing seeds from which oil has been extracted and which has, in the wet basis, a protein content of the order of thirty percent (30%) to sixty-five percent (65%).

Still another object of my invention is to utilize as an ingredient of an explosive a nitro-protein complex derived or obtained from a vegetable material composed of leguminous seeds from which oil has been extracted, and in the preferred embodiment of my invention, I utilize as such an ingredient the nitro-compounds derived from a vegetable material composed of soybean meal from which oil has been extracted.

Still another object of my invention is to utilize as an ingredient of an explosive the nitro-protein complex derived or obtained from a vegetable material from which oil has been extracted by a process which does not denature the protein.

Still another object of my invention is to utilize or employ as an ingredient of an explosive a nitrated vegetable product obtained by the nitra-

2

tion of the solid residual product of the commercial extraction of oil from vegetable oil-bearing materials, and comprising a nitrated protein-rich vegetable composition resulting from the nitration of a vegetable oil-free and undenatured protein-rich residual product.

Still another object of my invention is to utilize or employ in an explosive the nitrated vegetable product resulting from the nitration of the solid residual product of the commercial solvent extraction of oil from oil-bearing materials, and comprising a nitrated protein-rich, substantially oil-free and substantially undenatured composition.

15 Still another object of my invention is to utilize or employ in an explosive the nitrated product resulting from the nitration of the solid residual product of the commercial solvent extraction of oil from oil-bearing materials, and comprising a substantially oil-free, undenatured protein-rich product embodying or containing a nitrated protein-complex of the order of thirty per cent (30%) to sixty per cent (60%) of said product.

20 My invention is based upon the discovery that when an oil-bearing vegetable material or substance, such as hereinafter specified, from which oil has been extracted is subjected to a conventional nitrating process, a nitro-compound of the constituents of such substance is produced, and 25 this new product, of which nitro-protein complex is the main constituent, though not in itself an explosive, may be utilized to become a participant 30 of a powerful explosive when mixed with another explosive or with substances having explosive characteristics, and also on the discovery that 35 the introduction of my said nitro-compounds or the nitro-protein constituent thereto will increase the explosive energy or power of the substances with which it is mixed.

30 In accordance with my invention, I take a suitable quantity of meal, and preferably soybean meal, from which oil has been extracted, preferably in accordance with patents heretofore issued to me for such oil extraction, in processes 40 which do not substantially denature the protein of such meal. This meal thus embodies a substantially undenatured vegetable protein. The meal is preferably finely ground, and subjected to a conventional nitrating process, preferably by utilizing a nitrating mixture of forty 45 percent (40%) sulphuric acid (concentrated) and sixty per cent (60%) nitric acid (concentrated), operating at low temperatures. I thus procure 50 a material comprising a mixture of nitro-compounds, the chemical character and the propor-

tion of which mixture will depend upon the chemical analysis of the meal subjected to the nitrating process. When soybean meal, from which oil has as aforesaid been extracted, is employed, I procure nitrated meal embodying approximately fifty-six percent (56%) to sixty-two percent (62%) of a nitro-protein complex, twenty-six percent (26%) to eighteen percent (18%) of nitro-carbohydrate and three percent (3%) to four percent (4%) of nitro-cellulose, wet basis.

Tests of this soybean meal embodying such nitro-compounds have shown that it will with difficulty ignite upon contact with an open flame, and that it will not burn but will merely char when heated in a suitable dish to a high degree of heat, such as produced by a red, electric heating coil.

Cottonseed meal will, depending to some extent upon the analysis of the meal, produce a nitro-compound mixture comprising approximately forty-two percent (42%) of a nitro-protein complex, twenty-seven percent (27%) of nitro-carbohydrate and eleven percent (11%) of nitro-cellulose, on a wet basis.

Flaxseed meal will, depending to some extent upon the analysis of the meal, produce nitro-compounds approximately of forty-eight percent (48%) of a nitro-protein complex, thirty-two percent (32%) of nitro-carbohydrate and seven percent (7%) nitro-fibre.

The above-specified meals are three examples of what I shall hereinafter term an "edible-oil group" of suitable meals. Other members of this group are peanut meal, sesame-seed meal, mustard-seed meal, rape-seed meal and other oil-bearing seeds, nuts and germs from which oil is extracted for edible purposes, and which contain relatively high percentages of proteins.

It will be understood that the higher the percentages of protein in the initial meal, the higher the ratio of nitro-protein complex can be procured in the nitrated meal, and I therefore preferably employ a raw meal from which oil has been extracted and which has, in the wet basis, a protein content of the order of thirty percent (30%) to sixty-five percent (65%).

By dissolving the nitro-protein complex obtained by my invention in a weak alkaline solution, and by precipitation with dilute acetic acid, it is possible to separate the above complex from the other nitro-compounds existing in my nitrated meal. But, in view of the fact that these other nitro-compounds may constitute ingredients of explosive mixtures, I preferably do not separate the same, but utilize all the nitro-compounds existing in the meal or produced by nitration as a final product which will serve as an ingredient of an explosive as above specified.

When, however, my nitro-protein complex hereinabove referred to is dissolved in weak alkali, the precipitate obtained with dilute acetic acid is of bright yellow color.

In some cases a nitro-protein complex may be required to create a new explosive or for other uses, and in such cases my nitrated meal will be found to comprise the cheapest source of such a nitro-complex.

I have found that when my nitrated meal is mixed in proper proportions and by proper methods with other explosives, such as explosives of the nitroglycerine class, nitrated-aromatic class, ammonium, sodium or potassium-nitrates class, chlorates and perchlorates class, and nitro-cellulose class, a new explosive mixture is produced

of increased power and with new and desirable explosive characteristics.

When my oil-extracted meal is subjected to the conventional nitration process as hereinabove described, it is preferably subsequently washed with water to free the material from acid and is then dried to produce the ingredient-product hereinabove specified.

A basic product may be obtained by subjecting to ammonia vapors the above washed product in dried and pulverized condition. This basic product is characterized by a bright orange color.

Analysis of my nitrated meal shows that nitration has increased the nitrogen content to approximately sixteen percent (16%) from an initial two and seven-tenths percent (2.7%).

It is my belief that in view of the above changes in the characteristics, a new chemical composition is produced, or that the chemical character of the protein is changed.

It is my belief, also, that my nitrated meal has a nitrogen content which is higher than similar nitrated products of which I have knowledge.

I have found that my nitrated meal or nitro-compound has itself explosive characteristics when mixed in proper proportions with potassium chlorate or with ammonium or sodium nitrates, and this mixture may serve as an explosive ingredient of various explosives of the classes hereinabove specified.

My preferred method of mixing my neutral or basic nitrated meal with one or more of such ingredients as potassium chlorate, ammonium or sodium nitrates or substances having similar characteristics is to mix the ingredients together in the presence of water in order to obtain a plastic mass which may be dried into suitable shape or form for the use to which it is to be applied. In this event the step of drying the washed product may be omitted.

As a result of my experiments, I believe that the nitro-groups introduced by the nitration of my meal are in such molecular combination as to fulfill the requirements for a typical explosive of the class of organic nitrates; in fact, the decomposition of my nitrate meal takes place with the development of considerable heat.

In view of the fact that the nitrated product does not, after being subjected to the nitration as above specified, possess sufficient oxygen to permit it to explode, a product is produced which is safe to ship and otherwise handle.

In view of the increased nitrogen content of my improved nitrated meal, the final ingredient-product when mixed with various other explosives as above specified provides a substance by the use of which the nitrogen content in the mixed explosive may be desirably increased.

Having described my invention, I claim:

1. A high-explosive ingredient consisting of the nitrated solid compound resulting from the nitration of the substantially oil-free, substantially undenaturate solid product of the commercial solvent extraction of oil from the edible-oil group of oil-bearing seeds.

2. A high explosive ingredient consisting of the nitro-protein complex constituent of the nitrated compound resulting from the nitration of the substantially oil-free, substantially undenaturate product of the commercial solvent extraction of oil from oil bearing seeds, and the separation of the nitrated proteins therefrom.

3. A high explosive ingredient consisting of the nitrated solid compound resulting from the nitration of the substantially oil-free, substantially

undenaturate solid product of the commercial solvent extraction of oil from the edible-oil group of oil-bearing seeds, and containing protein-complex of the order of thirty per cent (30%) to sixty-five per cent (65%) of the entire product.

4. A high explosive ingredient consisting of the nitrated solid compound resulting from the nitration of the substantially oil-free, substantially undenaturate solid product of the commercial solvent extraction of oil from the edible-oil group of oil bearing seeds, and containing nitro protein complex of the order of fifty-six per cent (56%) to sixty-two per cent (62%) of the entire product and having the characteristic that it does not possess sufficient oxygen to cause said 10 nitrated compound to have inherent explosive qualities, is not ignitable upon heating to a high

degree of heat produced by a red hot heater and is ignitable with difficulty by contact with an open flame, but said product when mixed with inherently-explosive, oxygen-containing material 5 is explodable by conventional methods, and when so exploded, decomposition of the entire mixture takes place and is accompanied with the development of considerable heat.

5. The process of nitrating the substantially oil-free and undenaturate solid residual product of the commercial solvent extraction of oil from oil-bearing seeds, comprising the preparing and grinding of said residual product in finely-ground condition, and nitration of said finely-ground product with a nitrating acid at a low temperature.

MICHELE BONOTTO.